

July 10, 1923.

1,461,372

W. E. TRENT

## PROCESS OF TREATING ORE AND LIKE MATERIALS

Filed Feb. 21, 1920



## UNITED STATES PATENT OFFICE.

WALTER E. TRENT, OF WASHINGTON, DISTRICT OF COLUMBIA, ASSIGNOR TO TRENT PROCESS CORPORATION, OF WASHINGTON, DISTRICT OF COLUMBIA, A CORPORATION OF DELAWARE.

## PROCESS OF TREATING ORE AND LIKE MATERIALS.

Application filed February 21, 1920. Serial No. 360,452.

*To all whom it may concern:*

Be it known that I, WALTER E. TRENT, citizen of the United States of America, residing at Washington, in the District of Columbia, have invented certain new and useful Improvements in Processes of Treating Ore and like Materials, of which the following is a specification.

The invention relates to a process of sintering and smelting ores and materials in a fine state of division.

It is an object of the invention to provide a process for sintering and smelting finely divided ores and materials, by first forming a sintered mass of divided fuel and ore or other materials, and in secondly burning the fuel of the mass to smelt the ore or material incorporated therein.

The invention aims to provide a process for effectively treating fine particles of ore to smelt the same. It is also applicable to the treatment of that class of materials known as downtime or flue dust, slimes, sludge, precipitates and the like.

It is a further object of the invention to provide a process of smelting ore in a treatment chamber, wherein the use of refractory linings is eliminated in whole or in part by protecting the walls of the container with a portion of the sintered mass which constitutes a heat protecting lining therefor.

In following the process the finely divided ore is fluxed if necessary and both fuel and fluxed ore introduced to the treatment chamber under a desired velocity to be subjected to the proper heat treatment. The fuel may be comminuted coal, coke, fuel oil, a combustible gas, or the like. The heat treatment renders the charge in a somewhat viscous or sticky condition so that when projected with suitable velocity upon a surface, the charge will adhere thereto and build up a sintered and agglomerated mass. The entire charge is directed towards the wall of the treatment chamber, and the particles of ore together with that portion of the fuel which has not been burned are made to adhere to the same and to each other thereby removing the solids from the gaseous products which are then discharged.

Many ores and mineral substances contain combustible materials such as carbon,

sulphur, and the like, which render the addition of fuel unnecessary, or only necessary in less quantities, and in treating such substances the addition of extraneous fuel may be eliminated or curtailed.

The fuel substance, whether it be extraneous or inherent, will preferably be only partly consumed in forming the sintered mass as it is desirable to leave a sufficient amount of fuel distributed throughout the mass so that the smelting of the same may take place by introducing a proper supply of oxygen or air to the treatment chamber to cause combustion of the remaining fuel incorporated with the charge. At other times the fuel will be completely consumed in forming the sintered mass of partially smelted ore, and additional fuel will be added as required to complete the smelting of the sintered mass.

When a sintered mass has been formed, the same may be discharged and introduced to a smelting furnace of any well known type, or preferably, without removing the mass from the treatment chamber, the smelting operation can be finished by introducing a supply of air, or fuel and air to the chamber. The heated condition of the chamber and the charge, when the air is thus introduced, will result in a burning of the fuel and a smelting of the finely divided sintered and partially treated particles of ore. The part of the charge directly exposed to the heat, and thereafter progressively the balance of the mass becomes smelted forming slags and metal which collect in molten form and are discharged either continuously or intermittently.

The smelting reactions desired may require either an oxidizing, reducing or neutral atmosphere, and any of these conditions can be maintained, for example, when reducing iron oxide ores, only sufficient oxygen will be introduced so that part of all of the fuel will be converted into carbon monoxide, which gas will take oxygen from the iron oxide forming carbon dioxide gas and metallic iron. An example of an oxidizing atmosphere will occur in treating iron-zinc sulphide when desired to form  $SO_2$  and  $SO_3$  gases and metallic oxides or metals. In this case air will be introduced in sufficient quantities to convert the car-

bon fuel to  $\text{CO}_2$ , plus an additional amount to combine with the sulphur forming the sulphurous gases above mentioned.

In the accompanying drawings, I have shown a single embodiment of an apparatus for carrying out the process, but it will of course be understood that this disclosure is merely made for the purpose of illustration, and various forms of apparatus may be employed to support the process.

In the drawings, Figure 1 represents a longitudinal section of the apparatus.

In the smelting of ores, I have discovered that if the ore, or like material, in a fine state of division, is mixed with a fuel and slagging agent, and the charge given a heat treatment, a sintered mass can be formed consisting of, partially slagged ore, and fuel, in a relatively firm state. To form this sintered mass, it is preferable to project the heat treated particles of ore and fuel upon a surface when they are in an adhesive condition, at which time the charge will adhere to the surface, and the particles to each other, forming a coherent mass of ore and fuel in a sintered condition. It will, therefore, be seen that the sintered mass contains fuel and thoroughly distributed particles of ore so that to smelt the ore it is only necessary to consume or burn the fuel of the mass, the burning beginning with the exposed fuel, and progressively consuming the desired quantity of fuel in the mass which results in a smelting and slagging of the ore particles distributed therein. The burning of the fuel of the mass is preferably regulated so that combustion is terminated before the entire mass of sintered fuel and ore disposed within a treatment chamber is smelted in order to leave a sufficient thickness of charge to constitute a protecting lining for the chamber. This lining eliminates or curtails the necessity of using refractory linings which are now used in all types of smelters and must be frequently replaced, and if a refractory lining is used the coating of sintered charge will protect it from deterioration.

Referring now, more specifically to the drawings wherein like reference characters indicate corresponding parts the numeral 1 designates a treatment chamber which may be of any desired size and configuration but which for the purpose of illustration is shown as of a cylindrical shape having bell shaped ends and hollow supporting trunnions 2 and 3 at each end thereof. The chamber 1 is also provided with a removable top or cover plate 4, normally maintained in position by threaded members 5, and having an opening 6' therein adapted to be normally closed by a closure plate 7, movable to expose the opening when desired, for a purpose which will hereinafter appear. At one end the hollow trunnion 3

of the treatment chamber receives a slidably disposed feed member 6, having a discharge head 7' provided with peripheral discharge openings 8, the hollow shank of the feed member being connected at its opposite end with a threaded rod 9 disposed within the interior of a feed conduit 10 and operated by means of a hand wheel 11, connected therewith for reciprocating the feed member 6 within the treatment chamber. To enable a reciprocation of this feed member upon an actuation of the hand wheel 11, a nut 12 provided with threads cooperating with the threads on the rod 9 is employed, this nut being positioned between suitable confining elements, and adapted to be engaged by a shiftable device 13. This device when in the position disclosed in Figure 1, prevents a rotation of the nut which, of course, imparts to the feed member 6 a sliding movement upon the actuation of the wheel 11.

The feed conduit 10 communicating with the feed member 6 is provided with an extension 14, extending to the point 15 and having a communication with a feed supply pipe 16, receiving a fuel, ore and slagging agent from the hopper 17 by means of the feed conveyor 18 communicating with a venturi disposed in the feed supply 16 in advance of an air pump 19 for creating an air current through the feed supply pipe 16, the conduit 10 and feeding member 6. A suitable air valve 20 is disposed within the feed supply pipe 16 at a point adjacent the pump for the purpose of admitting the required quantity of air to the treatment chamber when a mass of material is undergoing treatment. There is also disposed within the feed supply pipe 16 a water or other agent introducing feed pipe 21 for conveying water, oil, or the like to the material passing through this feed supply pipe under velocity.

The discharge end or trunnion 2 of the treatment chamber 1 communicates with a discharge elbow 22, a suitable packing 23 being disposed at the point of connection between these elements, while the conduit 22 is provided with a universal union connection 24 with a discharge pipe 25, telescoping with a discharge pipe 26 having a turning gland connection 27 with a discharge 28. A suitable discharge 29 is also disposed within the elbow 22 adjacent the end of the trunnion 2, this discharge being normally closed by a plug 30, the purpose of the different discharge openings to more fully hereinafter appear.

When a supply of finely divided ore, is to be smelted, the same is fluxed if necessary and introduced with a fuel agent such as pulverized coal, oil or the like, and fed from the hopper 17 into the feed supply 16. The pump 19 is of course placed in operation,

forcing air under velocity through the feed pipe 16, which takes up or entrains the incoming fuel and ore at the venturi, carrying the same through the feeding pipe 14, the feed conduit 10, and the feeding member 6, discharging the fuel air and ore under velocity through the peripheral openings 8 in the head of the feed member toward the side walls of the treatment chamber 1. 5

10 Prior to the introduction of this fuel and ore the treatment chamber is preferably heated by means of a gas torch 31 the nozzle of which is inserted through the opening 6' normally closed by the closure plate 7 and this preliminary heating of the treatment chamber continues until the interior thereof has been heated to a temperature sufficient to ignite the fuel introduced to the chamber with the ore. Thereafter combustion 15 of the fuel mixed with the ore maintains the proper temperature in the treatment chamber to carry on the operation. When the desired temperature has been reached the torch is withdrawn and the heat 20 treatment occurs as a result of the combustion or partial combustion of the fuel introduced with the charge, all non-gaseous products from the fuel with the particles of ore which have become viscous and partially 25 smelted are projected against the inner surface of the treatment chamber and adhere thereto, and build up a sintered mass of carbon and partially smelted ore. The mass will firmly adhere to the walls of the treatment 30 chamber, or to the mass already formed, and the particles of ore and fuel will be uniformly distributed throughout the sintered mass. The feeding of the charge is continued until the desired thickness of the 35 sintered mass is built up on the inner surface to the treatment chamber, as disclosed for the purpose of illustration by the dotted lines in Figure 1. It is to be understood that while the charge is being introduced to the chamber and undergoing its heat treatment, the feed member 6 is slowly reciprocated or 40 moved by the manipulation of the turning wheel 11.

As shown in the drawings the trunnions 50 2 and 3 of the treatment chamber are supported in a cradle 31 for a rotary movement, the cradle being secured to a suitable supporting shaft having a gear 33 thereon, meshing with a worm 34, operated by a hand wheel 35. The supporting shaft has also a 55 loosely mounted pulley 36 disposed thereon, firmly connected with a sprocket 37 shown in dotted lines, the sprocket receiving a chain 38 turning over a sprocket 39 and 60 operating a worm gear 40 supported upon the cradle by means of a supporting shaft, the worm gear 40 meshing with a worm wheel 41 fixedly secured to the treatment chamber. By this construction it will be apparent 65 that during the formation of the sintered mass, the treatment chamber may be slowly rotated, so as to insure a uniform deposit of the mass upon the walls of the chamber, and this rotation is also very desirable during the smelting of the ore content in the mass which will be now described. 70

When a charge has been deposited upon the walls of the container, the removable cover 4 may be lifted from the treatment chamber or container, and the accumulated 75 mass broken up and removed from the container to be placed in a smelting apparatus for the smelting of the ore content distributed in the fuel. However, it is preferable not to remove the charge from the treatment chamber when the same is to undergo a smelting step, but rather to allow the charge to remain in the chamber during this operation when any fuel forming a part of the mass is consumed, or additional fuel supplied when sufficient fuel for proper smelting is not contained within the sintered mass. When a sintered mass is formed and the smelting of the ore is to take place, the hand wheel 35 is operated and through the 80 medium of the gears 33 and 34 the entire cradle and the treatment chamber is tilted for a reason which hereinafter appear. A sufficient quantity of air from the air pump 19 and valve 20 mixed with fuel if desired, 85 is introduced to the container of the treatment chamber and combustion brought about by the heat of the chamber and the exposed mass, causing a smelting of the mass. During the introduction of this air the treatment 90 chamber is slowly revolved by the mechanism which has heretofore been described. The air feed member 6 may also be reciprocated, the part of the charge directly exposed to the heat becoming 95 smelted, and thereafter the balance of the mass progressively smelted as the fuel is consumed. When a sintered mass is being formed in the treatment chamber, the products of combustion and any unburned distilled or volatile content of the fuel are discharged through the elbow 22 and discharge conduits 25, 26 and 28 to a point of collection 100 for the recovery of the unburned or partially burned gases, the same also applying 105 during the smelting step. The molten metal and slag, resulting from the smelting operation flows through the trunnion 2 and discharge opening 29 to a point of collection. During the smelting operation the cradle 110 and the treatment chamber can be tilted to any desired angle, so that the molten mass is discharged continuously as formed, intermittently, or at one pouring at the end of said operation. The treatment chamber is 115 then returned to a substantially horizontal position for the formation of another sintered mass. 120

When smelting the charge it is preferable to discontinue combustion of the fuel when 125 130

the sintered mass has been smelted to a point adjacent the walls of the treatment chamber, thereby leaving a film or layer of unburned fuel and ore which constitutes a heat protecting lining for the container.

This lining eliminates in whole or in part the need of using refractory linings, which in the case of other types of retorts require frequent replacements. When a new sintered mass is being formed in the treatment chamber, the same will readily accumulate upon the unburned film or layer of sintered fuel and ore remaining in the treatment chamber.

Having thus described the invention, what I claim is:

1. The method of treating ore and like materials, consisting in subjecting divided particles of ore or the like to heat treatment to place the same in adhesive condition, in projecting the treated ore upon a collecting surface to form a coherent mass, and in then applying heat to the mass to smelt the ore.

2. The method of treating ore and like materials, consisting in subjecting divided particles of ore and a fuel to a heat treatment to place the particles in an adhesive condition, and to distill the volatile products from the fuel, in projecting the heated particles upon a collecting surface to form a sintered composite mass, and in then causing combustion of the fuel in the mass, to smelt the ore contained therein.

3. The process of treating ore and like materials consisting in introducing to a treatment zone comminuted fuel and ore, in subjecting the fuel and ore to a heat treatment to place the particles in a viscous condition, in projecting the viscous particles upon a collecting surface to form a coherent mass, and in smelting the ore contained in the mass by burning the fuel thereof during a movement of the collecting surface.

4. The process of treating ore and like materials consisting in introducing to a treatment chamber comminuted fuel and ore, in subjecting the fuel and ore to the presence of heat to place the particles in a viscous condition and to distill the volatile content from the fuel, in projecting the viscous particles upon the chamber walls, in rotating the chamber, and in burning the fuel of the mass on the chamber walls during the rotation thereof.

5. The process of treating ore and like materials, consisting in introducing to a treatment chamber comminuted fuel and ore, in subjecting the fuel and ore to a heat treatment to distill the volatile products from the fuel, in projecting the heated particles upon the walls of the treating chamber to form a coherent mass thereon of fuel and ore, and in smelting the ore by introducing to the chamber oxygen to cause a burning of the fuel in the mass.

6. The process of treating ore and like

materials, consisting in introducing to a treatment chamber comminuted fuel and ore, in subjecting the fuel and ore to a heat treatment to distill the volatile products from the fuel, in projecting the heated particles upon the walls of the treating chamber to form a coherent mass thereon of fuel and ore, and in smelting the ore by introducing to the chamber oxygen to cause a burning of the fuel in the mass, and in moving the container during the combustion of the fuel collected on its wall.

7. The process of treating ore and like materials, consisting in introducing to a treatment chamber comminuted fuel and ore, in subjecting the fuel and ore to a heat treatment to distill the volatile products from the fuel, in projecting the heated particles upon the walls of the treating chamber to form a coherent mass thereon of fuel and ore, in smelting the ore by introducing to the chamber oxygen to cause a burning of the fuel in the mass, in moving the container during the combustion of the fuel collected on its wall, and in discontinuing the introduction of oxygen to the container when the fuel in the mass has been consumed to a point adjacent the collecting walls of the container.

8. The process of treating ore and like materials, consisting in introducing to a treatment chamber comminuted fuel and ore, in subjecting the introduced materials to a heat treatment to distill the volatile products therefrom and to place the solid particles in a viscous condition, in projecting the viscous particles upon a projecting surface of the container to form a coherent mass, and in then smelting the mass by introducing air to the chamber to cause combustion of the fuel of the mass.

9. The process of treating ore and like materials, consisting in introducing to a treatment chamber comminuted fuel and ore, in subjecting the introduced materials to a heat treatment to distill the volatile products therefrom and to place the solid particles in a viscous condition, in projecting the viscous particles upon a projecting surface of the container to form a coherent mass, and in then smelting the mass by introducing air to the chamber to cause combustion of the fuel of the mass, and in discontinuing the introduction of air to the chamber when the fuel in the mass has been consumed to a point adjacent the collecting surface to leave an unburned layer of material on said surface.

10. The process of treating ore and like materials, consisting in introducing to a treatment chamber comminuted fuel and ore, in subjecting the introduced materials to a heat treatment to distill the volatile products therefrom and to place the solid particles in a viscous condition, in pro-

40

45

50

55

60

65

- jecting the viscous particles upon a projecting surface of the container to form a coherent mass, and in then smelting the mass by introducing air to the chamber to cause combustion of the fuel of the mass, and in discontinuing the introduction of air to the chamber when the fuel in the mass has been consumed to a point adjacent the collecting surface to leave an unburned layer of material on said surface, and in rotating the container during the smelting of the formed mass.
11. The process of treating ore, which consists in subjecting to a heat treatment fine particles of ore and a carbonaceous fuel, in collecting the volatiles removed from the fuel, in projecting the carbonized fuel particles and the ore upon a collecting surface to form a coherent mass of the fuel and ore particles, and in then smelting the ore by burning the fuel distributed throughout the mass.
12. The process of treating ore, which consists in subjecting fine ore and coal particles to a heat treatment to place said particles in a viscous condition, and in projecting the viscous particles upon a collecting surface with sufficient force to cause them to unite to one another and form a composite mass of fuel and ore.
13. The process of treating ore, which consists in subjecting fine ore and coal particles to a heat treatment to place said particles in a viscous condition, and in projecting the viscous particles upon a collecting surface with sufficient force to cause them to unite to one another and form a composite mass of fuel and ore.
14. The process of treating ore and like materials, which consists in introducing to a movable collecting receptacle fine particles of ore and carbonaceous material, in heating the collecting receptacle to place said particles in a viscous condition, in projecting the viscous particles with sufficient force upon the rotating walls of the receptacle to cause said particles to unite thereon and build up a coherent mass of the fuel and ore, and in thereafter changing the condition of the ore by burning the fuel content in the mass.
15. The process of treating ore and like materials, which consists in introducing to a movable collecting receptacle fine particles of ore and carbonaceous material, in heating the collecting receptacle to place said particles in a viscous condition, in projecting the viscous particles with sufficient force upon the rotating walls of the receptacle to cause said particles to unite thereon and build up a coherent mass of the fuel and ore, and in thereafter changing the condition of the ore by burning the fuel content in the mass and by introducing to the rotating receptacle a supply of oxygen to promote the combustion of the fuel.

In testimony whereof I affix my signature.

WALTER E. TRENT.